

## UNITED STATES PATENT OFFICE

WILHELM LOMMEL, OF WIESDORF-ON-THE-RHINE; HEINRICH MÜNZEL, OF LEVER-KUSEN-ON-THE-RHINE; AND WINFRID HENTRICH AND MAX HARDTMANN, OF WIESDORF-ON-THE-RHINE, GERMANY, ASSIGNEES TO I. G. FARBENINDUSTRIE AKTIENGESELLSCHAFT, OF FRANKFORT-ON-THE-MAIN, GERMANY

## PROCESS FOR PROTECTING MATERIALS AGAINST ATTACK BY MOTHS

No Drawing. Application filed March 11, 1927, Serial No. 174,693, and in Germany March 15, 1926.

The present invention relates to a process for protecting materials against attack by moths and to the materials thus obtained.

In accordance with this invention the protection of wool, fur, hair and the like from attack by moths is effected by a treatment of the material in question with the esters of phosphoric acid, so that the same are uniformly incorporated within the materials and permanently retained therein.

According to our preferred mode of working the materials to be moth-proofed are immersed in solutions of the phosphoric acid esters in suitable solvents, as for example benzine, carbon tetrachloride, alcohols such as for instance ethyl and methyl alcohol, and the like, or they are sprayed with such solutions, or treated by some such process, which will serve to incorporate the desired moth-proofing ingredient, so that it will be retained thereafter. It will be understood that other carriers or diluents may be used.

The following examples will serve to illustrate the principles underlying our invention:

*Example 1*

The goods are immersed in a 2% solution of diphenyl-o-cresyl-phosphoric acid ester in benzine and after removal of the excess of liquid they are dried. The goods after the treatment are moth-proofed without detriment to the color and other physical characteristics.

*Example 2*

A 1% solution of triphenyl phosphoric acid ester in wood alcohol is sprayed upon the article to be mothproofed. After the evaporation of the alcohol the goods are fully protected against attack by moths.

In an analogous manner other esters of the phosphoric acid, such as the diphenyl- $\alpha$ -naphthyl ester, diphenyl- $\beta$ -naphthyl ester, diphenyl-o-, m- and p-cresyl esters, phenyl di-m-cresyl ester, tri-o-chlorophenyl-ester, tri-o- and p-chloro-phenyl esters, mono-phenyl-di-m-chlorocresyl ester, tetraphenyl-resorcylic ester, tricresyl ester or the like, or suitable mixtures of any two or more of these, can be applied. Such mixtures can be pro-

duced either by mixing the pure esters in any desired proportion or by producing mixtures of the esters directly from a mixed starting material such as for example crude cresol.

Other moth protecting agents, e. g., such as are described in our prior Patent No. 1,562,510 can also be admixed with the phosphoric acid esters, if desired.

We claim:

1. The process for protecting wool, furs and other materials against attack by moths, which consists in impregnating the material with a solution of a phosphoric acid aryl ester.
2. The process for protecting wool, furs and other materials against attack by moths which consists in impregnating the material with an aryl ester of phosphoric acid.
3. The process for protecting wool, furs and other materials against attack by moths which consists in impregnating the material with an alcoholic solution of diphenylcresyl-phosphoric acid ester.
4. Materials which are liable to attack by moths impregnated with an aryl ester of phosphoric acid.
5. Materials which are liable to attack by moths impregnated with diphenyl-cresyl-phosphoric acid ester.
6. As moth proofing agents, arylesters of phosphoric acid.
7. As moth proofing agents, solutions of arylesters of phosphoric acid.
8. As a moth proofing agent, an alcoholic solution of an arylester of phosphoric acid.
9. As a moth proofing agent, an alcoholic solution of triphenyl-phosphoric acid ester.

In testimony whereof we have hereunto set our hands.

WILHELM LOMMEL.  
HEINRICH MÜNZEL.  
WINFRID HENTRICH.  
MAX HARDTMANN.

90

95

100